

## UNITED STATES PATENT OFFICE.

ERNEST GUSTAV EDWIN MEYER, OF LONDON, ENGLAND.

## FUEL FOR USE IN INTERNAL-COMBUSTION ENGINES AND FOR OTHER PURPOSES.

No Drawing. Application filed June 5, 1926, Serial No. 114,021, and in Great Britain June 12, 1925.

This invention relates to fuels for use in internal combustion engines and for other purposes.

The object is to provide improved fuels containing considerable proportions of the higher boiling or less volatile or low grade hydrocarbon materials for use in the operation of internal combustion engines and particularly internal combustion engines of the character employed in the propulsion of road or marine vehicles.

Numerous proposals have been made with a view to achieving this object and certain of these have included the addition of an ether in order to facilitate the ignition and combustion of the fuel.

Hitherto it has been found that the employment of an ether is open to objection on a number of grounds.

For instance, the retention of the ether in the mixture is in some cases difficult and this has led to the addition of bodies intended to prevent the volatilization of the ether during storage and use.

In some cases phenolic bodies have been added to the fuel mixture for this purpose while in other cases where coal tar hydrocarbon distillates of the usual commercial grades have been used, the small proportion of phenolic bodies which they contain has acted in this direction. It would, however, appear to be due to the presence of these bodies in the known mixtures that difficulty has been experienced owing to the gumming of the valves and the formation of gummy or resinous deposits in the parts of the engine adjacent thereto.

One observation on which the present invention is based is that by the employment of alkali, and particularly ammonia, in the production of such ether-containing mixtures, certain advantages accrue; for instance, it would appear that the formation of a gummy or resinous mass in the gas passages adjacent to the valves and on the valves themselves may be largely if not entirely prevented by the treatment of these fuel mixtures.

The process of producing a fuel mixture adapted for use in internal combustion engines in accordance with the invention comprises, broadly, the introduction into a mixture consisting essentially of an ether and hydrocarbon distillates of a proportion of a

highly volatile basic material such as ammonia.

The introduction of the highly volatile material of a basic character may be effected by first preparing the mixture of an ether and hydrocarbon material and then treating it with a highly volatile basic material.

Alternatively the hydrocarbon material may be treated with a highly volatile basic material and the ether then added.

Ordinarily ammonia will be employed as the basic material.

Apparently the desirable results obtained are to be attributed to the retention of a proportion of the highly volatile basic material in the hydrocarbon and this may possibly be due to such materials containing a proportion of water.

On the other hand, it may be that a proportion of the highly volatile basic material, particularly if this be ammonia, is retained in solution in the hydrocarbon material itself.

Fuels in accordance with the invention in addition to ether may contain a proportion of constituents, usually hydrocarbons, of relatively low boiling point; for instance, the fuels may contain a proportion of hydrocarbon material boiling below 100° C. but not exceeding 25 per cent and the percentage of such constituents of low boiling point may be as low as 8 or 9 per cent.

Generally speaking, it is found that fuels containing between 9 and 22 per cent of constituents boiling below 100° C. are satisfactory.

Where the fuel is intended for use with internal combustion engines of the character employed in automobile vehicles, the end boiling point may be such that between 85 and 100 per cent of the material distils over 95 below 300° C.

Preferably the hydrocarbon material employed is such that 6 to 25 per cent distils over at temperatures up to 100° C., 30 to 60 per cent at temperatures up to 150° C., 50 to 98 per cent at temperature up to 200° C., and 86 to 100 per cent at temperatures up to 225 to 300° C.

As is well known the fuels adapted for use in internal combustion engines, of the type usually employed in the propulsion of automobile vehicles employing jet carburetors, contain a relatively considerable pro-

portion of hydrocarbon material which distils over below 100° C. and usually about 14 per cent or more distilling over at temperatures up to 80° C. For instance, the 5 standard No. 1 grade petrols which are sold in Great Britain at present contain a proportion of 40 per cent of material distilling over up to this temperature and a proportion of 14 per cent distilling over up to a temperature of 80° C. The remaining portion of such petrols usually distils over between the temperatures in question and about 185° C. or up to 200° C.

In order to obtain a fuel of this kind it is 15 considered necessary to enrich the straight fractions of certain crude oils boiling up to the maximum temperature above indicated, that is to say a temperature in the neighbourhood of from 185° C. to 200° C., by the addition thereto of material boiling below 100° C. derived from the treatment of further bodies of oil or crude oils of other origin.

Hydrocarbons boiling up to 85 to 90° C. possess a high commercial value, whereas 25 the mineral oil hydrocarbons boiling from 100 to 185° C. or above are of considerably lower value.

In order, however, to obtain a market for the latter grade of distillate, the more valuable distillates must be used in considerable 30 quantities.

Thus, the economical exploitation, that is to say, the exploitation of existing sources 35 of supply, of crude oil in order to produce the best financial results has hitherto been impossible of attainment in many cases.

A fuel according to the invention may consist essentially of a hydrocarbon distillate having an initial boiling point about 40 70° C. and a final boiling point between 150° and 225° C., in association with a small proportion of ether and a proportion of a highly volatile basic material.

Preferably the hydrocarbon material is of 45 such character that only 1 to 5 per cent passes over at 80°, from 12 to 25 per cent passes over below 100° C., and, for instance, 83 per cent at temperatures up to 150° C.

The final boiling point of the hydrocarbon material may vary between the limits 50 above stated according to the character of the oil; for instance, it may be found more convenient or economical to employ material which has a final boiling point between 55 175° and 225° C. and material having a final boiling point of 200° or even as low as 180° C. or 150° C. will in the majority of cases be available in sufficient quantity to render the use of such commercially practicable.

60 From the above it will be appreciated that the invention in certain of its preferred embodiments is distinguished from the majority of previous proposals in that the fuel is devoid of hydrocarbon material boiling below a temperature in the neighbourhood of

80° C. or contains a quite inconsiderable proportion of such material.

It furthermore may not comprise any considerable proportion of material boiling above 250° C. and rarely comprises more 70 than about 20 per cent.

The proportion of ether in fuel mixture in accordance with the invention is in all cases small, usually below 5 per cent, and in most cases it does not exceed 3 per cent.

The precise minimum boiling point of the hydrocarbon material employed may vary within the limits stated, as also may the proportion of the same which distils below a temperature of 100° C.

Normally hydrocarbon material boiling at a temperature not below 80° C., or of which merely 2 to 5 per cent distils over at 80° C., and of which 8 to 25 per cent distils up to 100° C., will be used.

The following particulars indicate the character of certain distillates which may be employed in accordance with the invention:—

| Temperature        | Percentage distilling over |    |      |      |    |    |    |
|--------------------|----------------------------|----|------|------|----|----|----|
|                    | A                          | B  | C    | D    | E  | F  | G  |
| Degrees centigrade |                            |    |      |      |    |    |    |
| 80                 | 0                          | 0  | 0    | 4    |    |    | 2½ |
| 90                 | 14                         | 12 | 12.5 | 12   |    |    |    |
| 100                | 34                         | 30 | 29   | 23.5 | 6  | 10 |    |
| 110                | 52                         | 46 | 47   | 39   |    |    |    |
| 120                | 65                         | 60 | 62   | 51   |    |    |    |
| 130                | 80                         | 72 | 75   | 64   |    |    |    |
| 140                | 87                         | 78 | 83   | 75   |    |    |    |
| 150                | 94                         | 85 | 90   | 83½  |    |    |    |
| 160                | 96                         | 90 | 94   | 90   | 50 | 60 |    |
| 170                | 98                         | 96 | 97   | 93½  |    |    |    |
| 180                | 99                         | 99 | 99   | 96½  | 70 | 90 |    |

The invention also extends as will be understood to the fuel mixtures produced by 105 the process.

The invention extends to fuel mixtures including coal tar distillates or mineral oil distillates or both.

By the expression "hydrocarbon materials 110 of higher boiling point," low grade distillates boiling above 160° C. and in some cases considerably above this limit, as well as the so-called low grade or No. 3 petrols which cannot normally be satisfactorily employed in the operation of relatively high speed internal combustion engines such as are used for the propulsion of automobile vehicles, are intended, while where hydrocarbon material of lower boiling point has been referred to, fractions distilling over completely at temperatures below 100° C. are meant.

As instances of materials adapted to be 115 employed as the main constituent of a fuel mixture, consisting mainly of hydrocarbons of relatively high boiling point, in accordance with the invention, the so-called white oils and gas oils may be mentioned.

The following particulars are given by 120

way of example to illustrate the composition of a fuel mixture in accordance with the invention consisting mainly of hydrocarbons of relatively high boiling point:—

- 5 87 parts by volume of a coal tar oil boiling between 160 and 260° C., 9 parts by volume of a petroleum hydrocarbon boiling below 100° C. and 4 parts of diethyl ether are mixed together and when completely mixed 10 a proportion of an alkali in solution is added and intimately mixed therewith.

As an example of the composition of a fuel mixture the following is given:—

- 15 96.5 parts of a petroleum fraction exhibiting a boiling range as follows:—8 to 12 per cent up to 100° C. and 85 to 100 per cent up to 300° C., are mixed with 3.5 parts of ethyl ether of s. g. 0.720 and the mixture treated with liquor or gaseous ammonia.

- 20 The concentration or proportion of the alkali employed would appear to be a matter of little importance while, as above indicated, the alkali may be employed in the proportion of 1 part of alkali to 10,000 parts of 25 the mixture.

While the invention is perhaps more particularly concerned with the production of fuels for internal combustion engines of the non-Diesel type, it is also concerned with 30 fuels for Diesel engines and fuels intended to be burnt in furnaces as, for example, in firing boilers.

Having now described my invention what I claim as new and desire to secure by Letters Patent is:—

1. A fuel for use in internal combustion engines and for other purposes, consisting essentially of hydrocarbon distillates in admixture with ether and a highly volatile 40 basic material.

2. A fuel for use in internal combustion engines and for other purposes, consisting essentially of hydrocarbon distillates in admixture with ether and ammonia.

45 3. A fuel for use in internal combustion engines and for other purposes, consisting essentially of hydrocarbon distillates and containing a small proportion of ether and as a highly volatile basic material.

50 4. A fuel for use in internal combustion engines and for other purposes, consisting essentially of hydrocarbon distillates and containing a small proportion of ether and ammonia.

5. A fuel for use in internal combustion engines consisting essentially of a hydrocarbon distillate, having an initial boiling point of about 70° C. and a final boiling point of about 300° C. and containing a small proportion of ether and a highly volatile basic 60 material.

6. A fuel for use in internal combustion engines consisting essentially of a hydrocarbon distillate, of which 1 to 5 per cent passes over up to 80° C., 8 to 25 per cent up to 100° 65 C., 20 to 65 per cent up to 120° C., and the balance boils at temperatures not substantially exceeding 320° C., and containing a proportion of ether, not exceeding one-twentieth of the volume of hydrocarbon 70 material, and a proportion of a highly volatile basic material.

7. A fuel for use in internal combustion engines consisting essentially of a hydrocarbon distillate, of which 1 to 5 per cent passes over up to 80° C., 8 to 25 per cent up to 100° 75 C., 20 to 65 per cent up to 120° C., and the balance boils at temperatures not substantially exceeding 320° C., and containing a proportion of ether, not exceeding one-twentieth of the volume of the hydrocarbon material, and a proportion of ammonia.

8. A fuel for internal combustion engines consisting essentially of a hydrocarbon distillate having an initial boiling point of 85 from 70 to 80° C. and of which not more than 5 per cent passes over up to 80° C., a final boiling point of not exceeding 320° C. and containing a small proportion of ether and a proportion of a highly volatile basic 90 material.

9. A fuel for internal combustion engines consisting substantially of 95 per cent of a hydrocarbon distillate of which not more than 5 per cent passes over up to 80° C. and 95 of which the balance is ether and a highly volatile basic material.

10. A fuel for internal combustion engines consisting of a hydrocarbon distillate, the main proportion of which boils below 160° 100 C., while a proportion thereof up to 5 per cent boils below 80° C., together with a small proportion of ether and a small proportion of a highly volatile basic material.

In testimony whereof I have signed my 105 name to this specification.

ERNEST GUSTAV EDWIN MEYER.